

1

3,594,174

NOVEL ANTIFOGGANT FOR SILVER HALIDE  
EMULSION ON A POLYESTER FILM SUPPORT  
Teruhide Haga, Koichi Horigome, Masao Ishihara, and  
Osakazu Sugino, Tokyo, Japan, assignors to Konishiroku  
Photo Industry Co., Ltd., Tokyo, Japan  
No Drawing. Filed Jan. 29, 1969, Ser. No. 795,034  
Claims priority, application Japan, Jan. 31, 1968,  
43/5,398

Int. Cl. G03c 1/34  
U.S. CL. 96—109

3 Claims

### ABSTRACT OF THE DISCLOSURE

A light-sensitive silver halide photographic material which comprises a polyester film support and, coated thereon, a light-sensitive silver halide emulsion, at least one layer of said photographic material containing a new antifoggant specified later. The said antifoggant prevents the impurities in the polyester film support from fogging the silver halide emulsion during its storage or incubation.

This invention relates to a light-sensitive silver halide photographic material which comprises a polyester film support and, coated thereon, a light-sensitive silver halide photographic emulsion, at least one layer of said photographic material containing a new antifoggant specified later.

Recently, polyester film has been brought into wide use as a support for a photographic element instead of cellulose triacetate film, because of excellent physical properties of the former. However, the polyester film disadvantageously contains a variety of byproducts, catalyst residues and other impurities, among which certain compounds usually cause very severe fogging on a light-sensitive silver halide photographic emulsion during its storage or incubation. Even if these byproducts, catalyst residues, etc. can be removed through an improved process for the production of polyester film, it is still unavoidable to prevent the self-decomposition of polyester with the result that the resulting decomposition products possibly cause increased fog on the emulsion. Thus, it is very difficult to remove any fogging factors from a polyester film support at the stage of its preparation. As the consequence, it becomes necessary for the preparation of a light-sensitive silver halide photographic material using a polyester support to incorporate a suitable antifoggant into various layers coated on the support, e.g. sub layer, inter layer, emulsion layer, protective layer, etc. Unfortunately, however, any antifoggant suited for this purpose has not yet been known.

It is accordingly one object of this invention to provide a light-sensitive silver halide photographic material with a polyester film support, said material being freed from fogging due to the action of the polyester film support. In order to accomplish this object, we have now found a new antifoggant which when incorporated into the sub layer, inter layer, emulsion layer and/or protective layer of a light-sensitive silver halide photographic material is highly effective to prevent fogging due to the action of a polyester film support of said material. The antifoggants used in the present invention can be represented by the general formula



wherein  $n$  is an integer of 0 to 7, R is a hydrogen atom or an alkyl group of not more than 17 carbon atoms, a phenyl group or a naphthyl group which may be substituted optionally with hydroxyl, carboxyl or sulfo groups, and M is an alkali metal or ammonium cation. Typical

2

antifoggants include the following compounds which are listed below only for illustration.



### SYNTHESIS OF THE COMPOUND 2

11.4 g. of n-hexyl aldehyde dissolved in 60 ml. of ethanol is added to 10.4 g. of sodium bisulfite dissolved in 100 ml. of water. The resulting mixture is allowed to stand overnight at room temperature and then heated under reflux on a water bath for 4 hours. The reaction mixture which is pale yellow and clear is distilled under reduced pressure. The white crystalline residue obtained is dissolved in a water-methanol mixture and then the solution is added with ether. The precipitate formed is collected by filtration and dried under reduced pressure. The white crystalline product is the Compound 2. Yield 9.5 g. M.P.  $>300^\circ\text{C}$ .

### SYNTHESIS OF THE COMPOUND 4

To 11 g. of sodium bisulfite dissolved in 150 ml. of water, 13.8 g. of 3,4-dihydroxybenzaldehyde is added, with stirring. The resulting solution is allowed to stand

overnight and then heated under reflux on a water bath for 5 hours. The reaction mixture is concentrated and the brown crystalline mass separated is taken up into 400 ml. of methanol. The resulting solution is heated under reflux and then filtered while it is hot. The filtrate is concentrated once again. The crystalline residue is washed with an ethanol-ether mixture and then dried in vacuo. The brown crystalline product is the Compound 4. Yield 9.9 g. M.P. >300° C.

Any one of the above-indicated compounds is added to a light-sensitive silver halide photographic emulsion at the proportion of  $5 \times 10^{-1}$  to  $5 \times 10^{-5}$  mole per mole of silver halide in the emulsion. Alternatively, the selected compound may be incorporated into an inter layer, sub layer and/or protective layer at the amount of  $10^{-1}$  to  $10^{-5}$  mole per square meter of the surface of the finished light-sensitive photographic material. Use of the compounds in the excess amount should be avoided, as this causes extraordinary fogging during storage or heat treatment of the emulsion. Light-sensitive silver halide photographic emulsions which may be employed in the present invention include any conventionally known ones, e.g. silver bromide, silver iodobromide, silver chloride, silver chlorobromide or the like emulsions. It should be noted that compounds of the above general formula where  $n$  is taken for more than 8 are substantially ineffective for the intended purpose.

New antifoggants disclosed in this application are entirely different in their chemical structure and function from any conventionally known inhibitors and stabilizers. The antifoggants can be used singly or in combination with the known inhibitors and stabilizers. Further, coloring materials, color formers, sensitizers, hardners or other known agents for a silver halide photographic emulsion also can be used together with the antifoggants disclosed herein.

Now the present invention will be explained in detail with reference to the following examples.

#### EXAMPLE 1

A light-sensitive gelatinous silver halide photographic emulsion, which contains 100 g. of silver iodobromide with the AgI content of 1.5 mil percent, is subjected to second ripening with gold sensitization. Immediately after completion of said second ripening, the emulsion is added with an aqueous solution of 1,2-benz-5-methyl-7-hydroxy-3,4,7a-triazaindene and an alcoholic solution of 1-phenyl-5-mercaptop-tetrazole and then with formalin and saponin. The resulted emulsion is divided into four portions, two of which are loaded with the Compound 2 and other two are not so. One of the unloaded emulsions is coated on cellulose triacetate film support. The remaining three portions are individually coated in polyester film support. After drying of the coated supports, there are obtained four light-sensitive photographic films which are then subjected to sensitometry according to the JIS method K-7604. The results of sensitometric tests are set forth in Table 1.

TABLE I

| Support              | Compound 2 per 60 g.<br>AgX (g.) | Immediately after preparation |                | Incubated at 55° C. under 5% RH for 5 days |                |
|----------------------|----------------------------------|-------------------------------|----------------|--------------------------------------------|----------------|
|                      |                                  | Fog                           | Relative speed | Fog                                        | Relative speed |
| Cellulose triacetate | 0.07                             | 100                           | 0.11           | 120                                        |                |
| Polyester            | 0.08                             | 95                            | 0.62           | -----                                      |                |
| Do                   | 0.2                              | 0.07                          | 100            | 0.16                                       | 110            |
| Do                   | 2.0                              | 0.07                          | 100            | 0.12                                       | 110            |

As apparent from the above, the film sample prepared by coating the unloaded emulsion on polyester film support suffers from very serious fogging during the incubation at 55° C. This means that 1,2-benz-5-methyl-7-hydroxy-3,4,7a-triazaindene and 1-phenyl-5-mercaptop-tetrazole are not effective against fogging resulting from

polyester film support. In contrast to this, use of the Compound 2 can minimize the fog during high temperature incubation as little as that which is observed in the conventional photographic film using cellulose triacetate support. Further, photographic properties of film samples just after their preparation indicate that the Compound 2 has no adverse influence on the properties. It is clear that the Compound 2 is effective against fogging due to the use of polyester film support.

10

#### EXAMPLE 2

A light-sensitive gelatinous silver halide photographic emulsion, which contains 100 g. of silver iodobromide with the AgI content of 1.5 mol percent, is subjected to second ripening with gold sensitization. After completion of said second ripening, the emulsion subjected to optical sensitization. This emulsion is then added with 1,2-benz-5-methyl-7-hydroxy-3,4,7a-triazaindene and then with formalin and saponin. The resulted emulsion is divided into four portions, two of which are loaded with the Compound 9 and other two are not so. One of the unloaded emulsions is coated on cellulose triacetate film support. The remaining three portions are individually coated on polyester film support. After drying of the coated supports, there are obtained four light-sensitive photographic films which are then subjected to sensitometry according to the JIS method K-7604. The results of sensitometric tests are set forth in Table 2.

TABLE 2

| Support              | Compound 9 per 60 g.<br>AgX (g.) | Immediately after preparation |                | Incubated at 55° C. under 5% RH for 5 days |                |
|----------------------|----------------------------------|-------------------------------|----------------|--------------------------------------------|----------------|
|                      |                                  | Fog                           | Relative speed | Fog                                        | Relative speed |
| Cellulose triacetate | -----                            | 0.09                          | 100            | 0.13                                       | 130            |
| Polyester            | -----                            | 0.10                          | 90             | 0.55                                       | -----          |
| Do                   | 0.2                              | 0.09                          | 95             | 0.14                                       | 125            |
| Do                   | 2.0                              | 0.09                          | 95             | 0.12                                       | 130            |

As apparent from the above, the film sample prepared by coating the loaded emulsion on polyester film support is entirely free from fogging during the incubation at 55° C.

#### EXAMPLE 3

A light-sensitive gelatinous silver halide photographic emulsion, which contains 100 g. of silver iodobromide with the AgI content of 5.3 mol percent, is subjected to second ripening with gold sensitization. Immediately after completion of said second ripening, the emulsion is added with 1,2-benz-5-methyl-7-hydroxy - 3,4,7a - triazaindene, formalin and saponin. The resulted emulsion is divided into four portions, two of which are loaded with the Compound 6 and other two are not so. One of the unloaded emulsions is coated on cellulose triacetate film support. The remaining three portions are individually coated on polyester film support. After drying of the coated supports, there are obtained four light-sensitive photographic films which are then subjected to sensitometry according to the JIS method K-7604. The results of sensitometric tests are set forth in Table 3.

TABLE 3

| Support              | Compound 6 per 60 g.<br>AgX (g.) | Immediately after preparation |                | Incubated at 55° C. under 5% RH for 5 days |                |
|----------------------|----------------------------------|-------------------------------|----------------|--------------------------------------------|----------------|
|                      |                                  | Fog                           | Relative speed | Fog                                        | Relative speed |
| Cellulose triacetate | -----                            | 0.08                          | 100            | 0.12                                       | 120            |
| Polyester            | -----                            | 0.09                          | 95             | 0.40                                       | -----          |
| Do                   | 0.4                              | 0.08                          | 100            | 0.12                                       | 125            |
| Do                   | 1.0                              | 0.08                          | 110            | 0.15                                       | 130            |

As apparent from the above, the film sample prepared by coating the loaded emulsion on polyester film support is entirely free from fogging during the incubation at 55° C.

**5**  
**EXAMPLE 4**

To an aqueous gelatine solution, formalin and saponine are added. Then this solution is divided into two portions, one of which is added with the Compound 8 and then coated on polyester film support, while the other is coated, without addition of the Compound 8, on polyester film support.

Separately, a light-sensitive gelatino silver halide photographic emulsion containing 100 g. of silver iodobromide with the AgI content of 1.5 mol percent is subjected to second ripening with gold sensitization and then added with an aqueous solution of 1,2-benz-5-methyl-7-hydroxy-3,4,7a-triazaindene and an alcoholic solution of 1-phenyl-5-mercaptopotetrazole and then with formalin and saponin. This emulsion is coated on the polyester film supports as prepared above. For comparison, the same emulsion is coated directly on cellulose triacetate film support to give a control sample.

The photographic films thus prepared are subjected to sensitometry according to the JIS-method K-7604. The test results are set forth in Table 4.

TABLE 4

| Support              | Interlayer                   | Immediately after preparation |                | Incubated at 55° C. under 5% RH for 5 days |                |
|----------------------|------------------------------|-------------------------------|----------------|--------------------------------------------|----------------|
|                      |                              | Fog                           | Relative speed | Fog                                        | Relative speed |
| Cellulose triacetate | None                         | 0.10                          | 100            | 0.14                                       | 120            |
| Polyester            | Gelatine without additive    | 0.12                          | 100            | 0.36                                       | -----          |
| Do                   | Gelatine with the compound 8 | 0.10                          | 105            | 0.15                                       | 120            |

As apparent from the above, the simple interlayer is not effective to prevent unusual fogging due to the polyester film support, whereas incorporation of the Compound 8 into the inter layer is satisfactory for the intended purpose.

## EXAMPLE 5

A light-sensitive gelatinous silver halide photographic emulsion, which contains 100 g. of silver iodobromide with the AgI content of 1.5 mol percent, is subjected to second ripening with gold sensitization. Immediately after completion of said second ripening, the emulsion is added with an aqueous solution of 1,2-benz-5-methyl-7-hydroxy-3,4,7a-triazaindene and an alcoholic solution of 1-phenyl-5-mercaptopotetrazole and then with polyethylene glycol (average molecular weight 2000), formalin and saponin. The resultant emulsion is divided into four portions, two of which are loaded with the Compound 1 and other two are not so. One of the unloaded emulsions is coated on cellulose triacetate film support. The remaining three portions are individually coated on polyester film support. After drying of the coated supports, there are obtained four light-sensitive photographic films which are then subjected to sensitometry according to the JIS method K-7604. The results of sensitometric tests are not forth in Table 5.

As apparent from the above, addition of the Compound 1 into the photographic emulsions is entirely satisfactory to prevent fogging due to polyester film support during high temperature incubation and normal storage.

**6**

This example shows application of the invention to a light-sensitive silver halide color-photographic material.

A compound of the formula



is formed into a 3% methanol solution. To a green-sensitive high sensitivity color photographic silver bromide emulsion, the above-mentioned solution is added in an amount of 30 cc. per liter of said emulsion. This emulsion is then incorporated with a solution prepared by dissolving in a 1 N caustic soda solution, 15 g. of the inner-type color photographic magenta color coupler 1-(4-carboxyphenyl)-3-(4-palmitoylamino-benzoylamino)-5-pyrazolone, and the pH of this emulsion is adjusted to 6.8 by means of citric acid. The thus prepared emulsion is added with the Compound 8 and then coated onto a polyester film support and dried. The resulting film is subjected to entirely the same test as in Example 1, together with a sample film to which the Compound 8 has been added. Provided that, in this case, the treatments are carried out according such ordinary procedures that the films are developed by use of a color developer containing diethyl-p-phenylenediamine and are then subjected to water-washing, bleaching, water-washing, fixing, water-washing and drying. As the result, it was found and follows from the aforesaid that the light-sensitive silver halide color photographic material containing Compound 8 according to the present invention was completely free from undesired fogging due to the polyester film support whereas the film without Compound 8 exhibited serious fogging.

45 What we claim is:

1. A light-sensitive silver halide photographic material comprising an emulsion layer and a polyester film support containing a compound of the general formula



55 where  $n$  is an integer of 0 to 7, R is a hydrogen atom or an alkyl group of not more than 17 carbon atoms, a phenyl group or a naphthyl group which may be substituted with hydroxyl, carboxyl or sulfo groups, and M is an alkali metal or ammonium cation, the compound

TABLE 5

| Support              | Compound 1 per 60 g. AgX (g.) | Immediately after preparation |                | Incubated at 55° C. under 5% RH for 5 days |                | After storage over 3 months |
|----------------------|-------------------------------|-------------------------------|----------------|--------------------------------------------|----------------|-----------------------------|
|                      |                               | Fog                           | Relative speed | Fog                                        | Relative speed |                             |
|                      |                               |                               |                |                                            |                |                             |
| Cellulose triacetate |                               | 0.10                          | 100            | 0.15                                       | 130            | 0.12 105                    |
| Polyester            | 0.12                          | 90                            |                | 0.80                                       |                | 1.13 -----                  |
| Do                   | 0.5                           | 100                           |                | 0.14 110                                   |                | 0.12 100                    |
| Do                   | 2.0                           | 0.09                          | 100            | 0.13 115                                   |                | 0.11 105                    |

being added in the proportion of  $5 \times 10^{-1}$  to  $5 \times 10^{-5}$  mole per mole of silver halide or in an amount of  $10^{-1}$  to  $10^{-5}$  mole per square meter of surface of the light-sensitive photographic material which compound prevents fogging of the layer containing silver halide.

2. A light-sensitive silver halide photographic material as claimed in claim 1, wherein the incorporation of said compound is realized in the sub layer, inter layer, and/or emulsion layer.

3. A light-sensitive silver halide photographic material

as claimed in claim 1, wherein it is a light-sensitive silver halide color-photographic material.

**References Cited**

**FOREIGN PATENTS**

5 1,341,010 9/1963 France ----- 96—109

NORMAN G. TORCHIN, Primary Examiner

10 W. H. LOUIE, JR., Assistant Examiner